

May 31, 1938.

A. F. STRACK

2,119,088

METHOD FOR PRODUCING FLAT BLANKS FOR ALUMINUM COOKING VESSELS

Filed Oct. 3, 1935

FIG. 1



FIG. 2



FIG. 3



INVENTOR  
ALBERT FRIEDRICH STRACK

By Emil Bönnelycke  
ATTORNEY

## UNITED STATES PATENT OFFICE

2,119,088

METHOD FOR PRODUCING FLAT BLANKS  
FOR ALUMINUM COOKING VESSELS

Albert Friedrich Strack, Suresnes, France

Application October 3, 1935, Serial No. 43,437  
In Germany October 11, 1934

4 Claims. (Cl. 29—148)

This invention relates to method for the manufacture of half-finished products for the production of aluminum cooking vessels, and more particularly to semi-manufactured products which are furnished with the final form as regards the bottom of the vessel, but have not been completed as regards the walls thereof, but at the same time incorporate in suitable amount and location the material necessary for producing the walls.

Specifically the invention relates to a method for producing a flat blank in connection with a marketable semi-manufactured product for the production of aluminum vessels, such as saucepans, frying pans, kettles or the like, in which the bottom of the vessel is furnished on the exterior with heat-accumulating projections, whilst the remaining parts of the vessel are flat on either side. The semi-manufactured product according to the invention, consists of a plate, which is preferably of circular form in plan, and is of such thickness as to make the same suitable for the subsequent production of the walls of the vessel by means of the usual tools in a stamping or pressing operation, and which is furnished over its central area on the one side with projections, such as studs or ribs, integral with the plate and increasing the heating surface thereof, and possesses about this central area, which forms later the bottom of the vessel, a marginal portion of suitable width which is flat on both sides.

The method of producing the semi-manufactured product consists in placing an aluminum plate, which is of considerably greater thickness than that ultimately possessed by the semi-manufactured product, and has been raised to a temperature approaching as closely as possible the melting point of the metal, on to a die, which is furnished with recesses open towards the top for the formation of the projections, and forcing the material into the recesses of the die by means of a suitable drop hammer or tup, the material thus forged being extended laterally to form a ductile sheet.

To perform the forging operation as described it is necessary for the impact face of the tup to be somewhat roughened, as otherwise the frictional resistance would be too small as regards the lateral extension of the material, and in consequence the material would take this path of smaller resistance instead of also penetrating into the die. The extent of the penetration into the die in relation to the lateral extension of the material may be regulated by the extent to

which the roughening of the tup is performed. At the same time, by reason of the roughening of the tup, the formation of craters is prevented on the upper face of the material above the recesses in the die, as the frictional resistance produced by the roughened surface prevents the material from flowing into the recesses too quickly. The roughness of the surface of the material caused by the roughened face of the tup may be readily removed afterwards by suitable treatment.

The piece of work is released from the die by compressed air which after each stroke of the tup is introduced from below through a series of passages into the single recesses or pockets of the die and maintains the piece of work in a floating condition until the next impact of the tup.

The means employed for carrying out the above process comprise a steel block, at the centre of which there is fitted firmly the die proper having the recesses or pockets determining the shape of the projections, which recesses communicate with each other by means of passages extending to the bottom of the die and grooves or channels in the said bottom. This system of passages is connected, through the steel block, with a feed passage through which there is supplied the compressed air for lifting the piece of work in the die.

The invention will be described more fully with reference to the accompanying drawing, in which

Fig. 1 shows, partly in section, a form of embodiment of a semi-manufactured product according to the invention, in which the projections comprise several circularly disposed series of conical studs surrounded by a supporting ring.

Fig. 2 shows diagrammatically in two longitudinal sections the die block employed for producing the semi-manufactured product according to Fig. 1.

Fig. 3 is a horizontal section, viewed from below, along the line III—III in Fig. 2.

In carrying out the process according to the invention an aluminum plate 1 of suitable thickness and diameter is placed on a steel block 2, in which there is firmly fitted a swage or die 3 of circular form and having a substantially conical periphery widening out towards the bottom, the fitting of this die preferably being performed by previously heating the block 2, so that after cooling it constitutes one piece together with the die 3. The die 3 possesses conical recesses or pockets 4, which correspond in number, shape and location with the projections 5 to 55

be formed on the piece of work and may be, for example, as shown in Fig. 1. The recesses or pockets 4 merge downwards into passages 6; which open out into the lower face of the die and 5 are interconnected by means of annular and radial grooves 7. The system of passages in the die 3 is connected by a plurality of passages 8 in the block 2 with the feed passage 9, which 10 communicates with a compressed air source (not shown) for supplying compressed air to lift the piece of work in the die. The upper portions 10 and 11 of the oppositely disposed walls of the die 3 and block 2 respectively are so embodied 15 that they permit of the formation of an annulus 12 on the piece of work.

Prior to its treatment the aluminum plate 1 is raised to a temperature which approaches 20 as closely as possible to the melting point of the metal, but which at the same time is sufficiently below this point that the metal will not melt by reason of the additional heat generated 25 by the forging process.

This mode of operation is based on recognition 30 of the fact that the aluminum, when the temperature has been raised in this way as near as possible towards the melting point, is so malleable under impact that it may be forced to desired extent into the recesses or pockets to form the projections, and at the same time also extended laterally. The plate 1 is accordingly acted 35 upon by a drop hammer, the tup of which possesses a sufficiently large and suitably striated or otherwise roughened surface, so that with the means illustrated in Fig. 2 there is produced the semi-manufactured product according to Fig. 1.

The apertures 13 in the annulus 12 necessary 40 for passage of the combustion gases from the furnace are bored or punched afterwards.

The lifting of the piece of work in the die takes 45 place by the free application of a compressed air connection to the mouth of the passage 9. This method of application is important insofar as a fixed connection on the block would not be able to withstand the heavy and repeated blows of the hammer.

The lifting of the work by compressed air, in 50 which connection the piece of work is lifted together with the weight of the hammer resting thereon, so that an even ejection takes place without deformation also in those cases in which 55 the work may not be located perfectly evenly in the die, also offers the additional advantage that the air thoroughly cleans the passages and the recesses after the piece of work has been removed.

Moreover it is also important to lift the work 60 after each blow of the hammer, as in this way the inherent force of acceleration is increased upon the next impact owing to the co-operation of the piece of work, which is caused to float by the compressed air, under its own weight. An important advantage also consists in the fact 65 that contact between the pieces of work and the heat-dissipating surfaces of the die 2 is avoided between each two strokes of the hammer, an undue cooling of the work thus being prevented.

What I claim as new and desire to secure by Letters Patent is:

1. A method of producing a flat blank for an 70 aluminum cooking vessel having the bottom portion of the vessel finished in the blank and the side wall material adjacent thereto, comprising

placing a heated aluminum plate, which is of greater thickness and smaller diameter than the finished blank, on a block having a die therein corresponding to the bottom portion, and repeatedly subjecting the plate to forging blows by a 5 forging tool at the same time lifting the plate from the block between each of the forging blows until the plate is forged to the desired diameter to include the side wall material of the finished vessel and the bottom portion has received the desired configuration corresponding to that in the die, said forging step being carried out by the application of a varying frictional resistance in order to regulate the ratio 10 between the displacement of the metal to form the desired configuration of the bottom portion and the lateral extension of the side wall material.

2. A method of producing a flat blank for an 20 aluminum cooking vessel having the bottom portion of the vessel finished in the blank and the side wall material adjacent thereto, comprising placing a heated aluminum plate, which is of greater thickness and smaller diameter than the 25 finished blank, on a block having a die therein corresponding to the bottom portion, and repeatedly subjecting the plate to forging blows by a forging tool and applying air under pressure below the plate in order to lift the plate from the die immediately following each forging blow 30 until the plate is forged to the desired diameter to include the side wall material of the finished vessel and the bottom portion has received the desired configuration corresponding to that in the die.

3. A method of producing a flat blank for an 35 aluminum cooking vessel having the bottom portion of the vessel finished in the blank and the side wall material adjacent thereto, comprising placing a heated aluminum plate, which is of greater thickness and smaller diameter than the 40 finished blank, on a block having a die therein corresponding to the bottom portion, and repeatedly subjecting the plate to forging blows by a forging tool and forcing air under pressure 45 between the plate and the block in order to lift said plate together with the forging tool immediately following each forging blow until the plate is forged to the desired diameter to include the side wall material of the finished vessel and the bottom portion has received the desired configuration corresponding to that in the die.

4. A method of producing a flat blank for an 55 aluminum cooking vessel having the bottom portion of the vessel finished in the blank and the side wall material adjacent thereto, comprising placing a heated aluminum plate, which is of greater thickness and smaller diameter than the 60 finished blank, on a block having a perforated die therein corresponding to the bottom portion, and repeatedly subjecting the plate to forging 65 blows by a forging tool at the same time lifting the plate from the block between each of the forging blows until the plate is forged to the desired diameter to include the side wall material of the finished vessel and the bottom portion has received the desired configuration corresponding to that in the die in which projections are produced on said plate at the points of the perforations in the said die.